

May 8, 1934.

A. A. HANDLER

1,957,499

METALLIC PROPELLER AND METHOD OF MAKING

Filed Aug. 19, 1929 3 Sheets-Sheet 1



Fig. 1



Fig. 2



Fig. 3



Fig. 4

Inventor

ALFRED A. HANDLER.

By

Riley & Watts.

Attorneys

May 8, 1934.

A. A. HANDLER

1,957,499

METALLIC PROPELLER AND METHOD OF MAKING

Filed Aug. 19, 1929

3 Sheets-Sheet 2



INVENTOR  
ALFRED A. HANDLER

BY *Rickey & Watts*

ATTORNEY

May 8, 1934.

A. A. HANDLER

1,957,499

METALLIC PROPELLER AND METHOD OF MAKING

Filed Aug. 19, 1929

3 Sheets-Sheet 3



INVENTOR  
ALFRED A. HANDLER  
BY *Richard & Watts*  
ATTORNEY

## UNITED STATES PATENT OFFICE

1,957,499

METALLIC PROPELLER AND METHOD OF  
MAKINGAlfred A. Handler, Cleveland, Ohio, assignor to  
Aluminum Company of America, a corpora-  
tion of Pennsylvania

Application August 19, 1929, Serial No. 387,016

35 Claims. (Cl. 29—156.8)

This invention relates to the art of propellers and is particularly associated with certain novel methods for manufacturing propeller products.

Present day manufacturing methods are lacking in any processes for working individually the metal of the hub portion of a propeller. The known methods are also devoid of any steps for providing axial recesses in the propeller hub. A construction including a wrought hub perforated 10 by an axial recess is advantageous in aeronautical propellers as it lightens the article and yet leaves it with the properties of strength, toughness, etc., to the degree necessary to withstand severe service. Propellers made by conventional methods 15 are characterized by a hub portion of metal which has not been worked as much as the metal of the blade portion. This is because the latter has been thinned out more than has the hub. In order for the metal of the hub to exhibit the characteristics 20 of hot wrought metal to the extent desired, it is essential that the original ingot, from which it is formed be reduced in cross-sectional area sufficiently to bring about the change in the characteristics of the metal. In the case of an 25 aluminum base alloy a reduction of about 75% or more is necessary for proper results. It is, therefore, necessary to start with an ingot having a comparatively large diameter in order to obtain this reduction in the hub.

30 In view of the foregoing this invention has as an object the broad proposition of providing methods for working the metal of the hub portion of a propeller individually and which working is not necessarily accompanied by a working 35 of the blade portion. Such a method has the advantage of permitting the manufacturing of the product to begin with an ingot of much smaller cross-sectional area than has formerly been the case, and yet provide a hub portion that 40 is characteristically wrought. It further provides for the forming of the hub into a lightened construction such as by being recessed axially by the blade. Moreover, the individual working of the hub constitutes a method whereby the flow 45 lines of the metal of the hub portion may be made to conform to the contour thereof.

This last mentioned feature provides for a greatly improved hub portion as the conformity of the flow lines to the contour renders the construction more resistant to the stresses encountered in propeller use.

The individual metal working processes for the hub portion may take the form of metal upsetting, displacing or similar working operations. 55 Such methods serve to cause the metal to assume

the characteristics of wrought metal and also bring about a desired change in the shape of the hub portion. These operations are all closely related and simulate one another because the worked metal has substantially the same properties and qualities for propeller purposes. 60

More specifically, I propose to pierce the hub portion of a propeller while it is confined in dies of suitable shape. Such a piercing operation provides a recessed hub and is particularly adapted 65 to the forming of a desired hub structure, such as outstanding flanges.

This invention also involves the combination of metal working processes for the hub portion of a propeller with other propeller manufacturing 70 steps. It is my idea to provide a method including the individual working of the hub and also rolling out processes, forging by dies, pressing, finishing and heat treating.

More in detail, I intend to pierce the hub portion of a blade in a series of steps in order to upset or spread the metal thereof. This piercing ordinarily will follow the rolling and forging operations or it may be associated with pressing processes. These piercing operations involve the use 75 of confining dies into which the metal is upset. The latter are so dimensioned relatively to one another that the change in the shape of the hub is a more or less gradual one. This also provides for a thorough working of the metal crystals 80 as the deforming forces have a prolonged period of application.

In addition to the foregoing, other more detailed objects and advantages will in part become apparent and in part be hereinafter stated as the 90 description of the invention proceeds. For a full and more complete understanding thereof, reference may be had to the following description and accompanying drawings, wherein,

95 Figure 1 is a perspective view of a billet of metal before it is subjected to the processes of this invention.

Figure 2 is a view similar to Figure 1 showing the billet as it is formed by the first rolling step.

100 Figure 3 is a plan illustration of a propeller after it has been roughly shaped by the rolling operations.

Figure 4 is a diagrammatic showing of the forging rolls.

105 Figure 5 is a sectional view through a part of the piercing apparatus.

Figure 6 is a showing similar to Figure 5 and develops a more advanced step in the upsetting process.

Figure 7 is a view similar to Figures 5 and 6 and brings out the final piercing operation.

Figures 8, 9 and 10 are sectional views taken about on the lines 8—8, 9—9 and 10—10 of Figures 5, 6 and 7, respectively.

Figure 11 is a plan view of a propeller after it has been shaped by the rolling out and upsetting processes, and,

Figures 12, 13, 14 and 15 are sectional views taken about on the lines 12—12, 13—13, 14—14, 15—15 of Figure 11.

I wish to emphasize that my novel methods are designed to shape propeller blades from any of the metals or their alloys that have been found suitable for such use. In addition to an aluminum base alloy, which is taken for exemplary purposes as a preferred material to be fashioned into propeller shape, the following metals are mentioned among others as being susceptible to working by the method hereof: magnesium and the various magnesium base alloys, iron and steel, copper, and in its several combined forms, such as bronze and brass, and nickel in alloy compositions such as Monel metal. I wish to note particularly that the magnesium base alloys are peculiarly adapted for the making of aeronautical propellers. Such alloys exhibit many of the properties of aluminum base alloys and are desirable for the same reasons as are the latter. An aluminum base alloy which has been found suitable for aeronautical propeller use is one containing approximately ninety-four percent aluminum, four and five-tenths percent copper, seventy-five hundredths percent manganese, and seventy-five hundredths percent silicon.

A propeller blade such as made by the instant methods is described as being designed for use in gaseous fluids. This because blades for aircraft purposes must have all of the properties of strength, toughness and the like, to the highest degree necessary and still be as light as is feasible. These conditions are, to a certain extent, peculiar to aircraft and the improved methods are herein set forth as applied to aeronautical propeller manufacture. It is obvious, however, that the invention would be employed in the making of propellers that operate in other fluids, such as water.

In the present embodiment the propeller is made from an aluminum base alloy of the composition hereinbefore set out.

Referring now to the drawings, a metal billet that indicates the starting point of my method is shown in Figure 1 and designated A. The true starting point of the method is a cast ingot. Whether or not this has been worked down to the form of a billet as shown or remains in ingot form is immaterial to this invention. The method must begin somewhere with a casting and any methods starting out from a worked billet merely presume the prior working of the ingot into the billet form. The exact metal working operations which are availed of to reduce the ingot to billet form are not essential to this invention. A preferred method might include rolling out processes for this step which may be carried out in a blooming mill. This billet A is formed with a handle portion or tong hold 1 in any preferred manner. This portion 1 constitutes a means which is gripped by a pair of tongs or like tool to handle the billet during the operations to be hereinafter described.

The billet A is first heated to a condition wherein it is easily workable, for instance, to a temperature of about eight hundred twenty degrees F. It is then subjected to the action of forging rolls

indicated diagrammatically in Figure 4 as R. The rolling out operations preferably comprise a series of rolling steps or passes through the rolls R, which gradually work the billet A into the form shown in Figure 3 and impart to it the approximate sectional arc of a finished propeller. At this point the billet has taken on the general shape of a propeller and for the purposes of this description is referred to as B. The showing of Figure 2 develops the billet A after it has been deformed by the first rolling out step.

The rolling out operations provide, in somewhat rough form the blade B having a hub portion H. The metal in the blade portion will have been worked sufficiently to effect a reduction in its cross-sectional area of about seventy-five percent or more. If the reduction has not been carried out to this extent in the blade portion by the rolling out steps it will be completely effected by the subsequent forging or pressing operations, or both. However, the latter do not materially affect the hub portion H, so if the metal thereof has not been reduced to the critical point of about seventy-five percent reduction by the rolling out processes this will be attained by the subsequent hub working operations.

The rolling out steps impart to the metal a fine grained structure which is characterized by flow lines that conform in direction to the contour of the blade. A flow line in a wrought metal bears a certain relation to fiber in wood and the term "fiber" has come into quite common usage in the wrought metal field. It has been defined as a condition of parallelism of lines or structural details and may frequently be found in any wrought metal. On visual examination it may show itself through undissolved constituents, segregations, or non-metallic inclusions. Grains may quite often be found to be elongated in the direction of the fiber and the fiber will parallel the direction of the previous working.

Fiber or flow lines as I term them, may sometimes be visible to the unaided eye when a specimen of wrought metal is deeply etched, or may be apparent only on microscopic examination. Going even further, certain types of flow lines caused by preferred orientations of crystal axes are only distinguishable by X-ray analyses.

Intimately associated with the flow line arrangement as a part thereof is any laminated structure which may be caused by the presence of voids, dross, impurities and the like. Such laminations will be elongated lengthwise of the blade by the rolling and will assume the directions of the flow lines. Moreover, the size of the grains varies in a uniformly progressive manner with the thickness of the blade and the working received by the metal. Concentration or localization of voids, impurities, etc. in transverse relation to the propeller is also prevented by the rolling out. Such concentration of the voids ordinarily would result in a blistering or surface cracking of the metal. These features clearly demonstrate the desirability of the rolling out steps in comparison with the present day practice of hammering out the blade.

After the blade B has been roughly shaped by the rolling out steps it is again heated to a workable condition whereupon it is subjected to the action of forging dies. The latter are effective for the main part only on the blade portion proper and affect the hub portion H only by bringing it into a round shape such as indicated by dotted lines in Figure 5. The hub portion H will have been brought into substantially the

shape shown by the rolling operations and the forging by dies only affects it slightly. The forging operations preferably comprise a series of steps which gradually form the blade into what 5 is practically its finished shape.

If desired, the shaping by forging may be dispensed with wholly or in part and pressing operations substituted therefor. My thought is, however, that a complete manufacturing method may 10 include both of these processes. As in the case of forging, the blade is first heated to a point where it is workable and it is then subjected to the pressing dies. The action of the latter is characterized by the prolonged or continued application 15 of the deforming force. This metal working action simulates the rolling out steps in this respect and also the upsetting operations, to be later described.

The metal working operations for further 20 shaping the propeller after it has been rolled out are, for the purposes of this description, classified generally as forging. This term is intended to include all the metal working methods which 25 function to form, shape, or work the metal by applying a deforming force thereto. Such methods may comprise forging by dies and pressing as above noted.

Subsequent to the forming of the blade portion 30 by rolling and forging, or pressing, or both, which operations have shaped the hub portion H into a somewhat cylindrical shape, the handle portion or tong hold 1 is removed in any convenient manner as by cutting. The hub portion is then deformed, preferably by a series of piercing operations 35 which upset the metal of the hub portion. It is to be clearly understood that I am not to be confined to the exact upsetting operations disclosed because obviously equivalent processes could be availed of to attain the same ends.

40 In order to render the metal of the hub more easily workable, it is preferably heated to a proper point. The hub end of the blade is then introduced to the split die 2 shown in Figure 5 which closes and grips the hub. The latter is 45 formed with grooves and ribs 3 which define the shape of certain hub structure in the form of ridges and grooves which are to be present in the ultimate product. When the blade is first positioned in the die 2 the metal of the hub portion 50 occupies the position indicated by the dotted lines in Figure 5.

A piercing tool 4 having a point 5 is now operated by proper force and pierces the hub portion of the blade axially. This piercing of the 55 blade upsets the metal thereof so that it completely fills the space between the die 2 and piercing tool 4.

The blade is now removed from the die 2 and 60 introduced into the die 6. The action of the die 2 and piercing tool 4 has been to deform the metal of the hub to a shape resembling its final form. The die 6 and piercing tool 7 are designed to still further carry out this deformation. When 65 first positioned in the die 6 the hub H assumes the dotted line position. The tool 7 is then operated so that its point 8 pierces the hub by first entering the opening formed by the point 5. The metal is upset by this operation and displaced into the grooves 9 formed in the die 6. The hub 70 portion of the blade will now have more nearly reached its ultimate formation.

While two or even one piercing operation may 75 be found to be sufficient to properly form the hub of the finished blade, I propose to avail of three of these operations. It is evident that the up-

setting may be broken up into as many operations as found desirable under any particular circumstances.

After the tool 7 has been cleared away from the blade it is removed from the die 6 and introduced into the final die. Grooves 11 and rib 12 in the latter define the final hub structure. A piercing tool 13 having a point 14 is operated in the usual manner as above described and the metal of the hub H is upset from the dotted line position into the space between the die 10 and tool 13.

80 It is notable that the exact metal flowing action imparted to the metal of the blades by piercing is dependent on the size and shape of the piercing tool and confining die. Under proper dimensioning of these parts the metal will be both upset and caused to flow axially by this piercing. Such action is incorporated in the operations above outlined, but it is to be remembered that the piercing may upset the metal without axial flowing and vice versa.

85 While the point 5 is of a substantially round shape, the point 8 is flattened out somewhat and the point 14 even more so. These points provide 90 the openings 15, 16 and 17 shown in Figures 8, 9 and 10, respectively, during the several piercing steps.

95 While the hub portion has been finally shaped, the blade is subjected to the usual finishing operations, comprising cleaning, sizing, trimming and heat treating, and final finishing which may include polishing and trimming.

100 The upsetting or flowing of the metal of course changes any cast characteristics remaining inherent thereto after rolling to those of hot wrought metal. The final product is remarkably free from any irregular grain structure and coarse grains, and it is notable that the grains assume flow lines conforming in direction with 110 the contour of the propeller. Furthermore, it is characteristically wrought throughout and the hub portion is very light and yet of sufficient strength to meet the service conditions it will be 115 subjected to.

120 What I claim is:

1. In propeller manufacture, the method of shaping the hub portion of a propeller and root portion of the blade which lies in forming the hub portion into its final shape by a series of 125 piercing operations extending into the root portion of the blade.

2. The method of making a propeller blade, which comprises rolling a piece of metal out into general blade shape, and then working the hub 130 portion and root portion of the blade into finished form by axially piercing the metal thereof.

3. The method of making a propeller blade which consists of working a piece of metal into rough propeller shape, forming the hub portion 135 of the blade with a hollow, and carrying out the said working and forming operations to create a flow line arrangement in the grain structure of the hub portion of the blade conforming with the longitudinal contours of the propeller.

4. In propeller manufacture, the method of working a piece of metal down to a rough blade shape, having blade and hub portions, and carrying out the working to provide a longitudinal recess extending through the hub portion into 145 the blade portion and at the same time creating a grain structure in which the grains vary in size uniformly throughout the said blade and hub portions.

5. In the making of metallic propellers, the 150

- method which consists in applying a deforming force to a piece of metal to cause the latter to roughly assume the shape of a propeller blade having a hub portion, prolonging the time of application of the force to thoroughly work the crystals of the metal, and then working the hub portion by upsetting the metal thereof. 80
6. In the making of metal propellers, the method which consists in deforming a piece of metal into rough blade shape with the grain structure of the metal having flow lines conforming in direction to the contour of the blade, the blade being formed with a hub portion, and then deforming the latter to provide a hollow therein and working the metal thereof to a condition wherein the flow lines conform to the contour of the hub portion. 85
7. In propeller manufacture, the method which comprises forming a piece of metal into the general shape of a propeller blade, having hub and blade portions, further shaping the blade portion by forging, and then upsetting the hub portion into its final shape. 90
8. In propeller manufacture, the method which comprises forming a piece of metal into the general shape of a propeller blade, having hub and blade portions, further shaping the hub and blade portions by forging and pressing processes and then deforming the metal of the hub portion by upsetting operations. 95
9. In propeller manufacture, the method which comprises forming a piece of metal into the general shape of a propeller blade, having hub and blade portions, continuing the shaping of the blade by pressing processes, and then finally forming the hub portion by a piercing operation. 100
10. In the making of metal propellers, the method which consists of rolling a billet of metal out into the rough shape of a propeller blade, having a hub portion, further shaping the blade by forging, and then axially piercing the end of the hub portion of the blade to spread the metal thereof and provide a hollow hub portion. 110
11. In the making of metal propellers, the method which consists of rolling a billet of metal out into the rough shape of a propeller blade, further shaping the blade by forging, and then operating on the hub portion of the blade with a series of piercing operations, which gradually work the metal of the hub into its ultimate form. 115
12. In the making of metal propellers, the method which consists of rolling a billet of metal having the characteristics of cast metal out into the rough shape of a propeller blade, further shaping the blade by forging, and then working the hub portion of the blade to effect a reduction of the metal sufficient to change the characteristics thereof from those of cast metal to those of wrought metal. 120
13. In the making of metal propellers, the method which consists of rolling a billet of metal having the characteristics of cast metal out into the rough shape of a propeller blade, further working the metal of the hub portion to effect approximately a seventy-five percent reduction in the cross-sectional area of the hub portion. 125
14. The method of making a propeller blade which consists in heating a billet of an aluminum base alloy and working the billet while heated into a blade shape having hub and blade portions, and then forming the hub portion into a shape having a recess extending lengthwise of the propeller. 130
15. The method of shaping the hub portion of a metal propeller which consists in first forming a round hole in the hub portion, and then elongating the hole and forming the elongated portion of the hole in a flattened out shape. 135
16. The method of forming the hub portion of a propeller and root portion of the blade which comprises piercing the metal of the hub and blade axially to provide an opening therein, and then performing further piercing operations to change the shape of the hub portion, and to lengthen the opening therein. 140
17. In propeller manufacture, the method which consists in rolling out an aluminum base alloy billet to provide hub and blade portions and then working the said portions by a series of piercing operations to form a flattened out recess in the blade portion. 145
18. In the making of metal propellers, the method which lies in deforming a piece of metal into the rough shape of a blade having a hub portion, and then upsetting the metal of the hub portion by a series of piercing operations to provide a recess therein and also an outwardly extending flange. 150
19. In propeller manufacture, the method which comprises working a piece of metal while heated into the general shape of a blade having a hub portion, further shaping the blade by forging, and then gradually working the hub portion into its ultimate shape by a series of upsetting operations. 155
20. In propeller manufacture, the method which comprises working a piece of metal while heated into the general shape of a blade having a hub portion, further shaping the blade by forging, while the metal is in a heated condition, and then performing a series of piercing operations axially on the hub portion to provide a recess therein. 160
21. In the making of metallic propellers, the method which comprises rolling out an aluminum base alloy billet while in a heated condition to provide a blade in rough shape, having a hub portion, further shaping the blade by forging, and then axially piercing the metal of the hub portion. 165
22. In the making of metallic propellers, the method which comprises rolling out an aluminum base alloy billet while in a heated condition to provide a blade in rough shape, having hub and blade portions, further shaping the blade by performing forging and pressing operations while the blade is in a heated condition, and upsetting the metal of the hub and blade portion by a longitudinal piercing operation. 170
23. In propeller manufacture, the method of making a metal blade which consists of rolling out a metal billet while in a heated condition, forging the rolled out metal into a blade shape having a cylindrical hub co-axial with the blade, and then forming an axial recess in the hub. 175
24. In propeller manufacture, the method of making a metal blade which consists of rolling out a metal billet while in a heated condition, forging the rolled out metal into a blade shape having a cylindrical hub, and then upsetting the metal of the hub into a shape characterized by a flattened recess extending axially of the blade. 180
25. In propeller manufacture, the method of making a metal blade which consists of rolling out a metal billet while in a heated condition, forging the rolled out metal into a blade shape having a cylindrical hub, piercing the metal of the hub by a series of piercing operations to pro- 185

vide an outwardly extending flange thereon, and then carrying out finishing operations to provide the final product.

26. The method of making a propeller blade which consists in heating a metal billet to a workable condition, rolling out the metal while heated, forging the metal into propeller shape while in a heated condition, and which shape is formed with a hub portion, and then piercing the hub to provide a recess extending axially of the blade.

27. The method of making a propeller blade which consists in heating a metal billet to a workable condition, rolling out the metal while heated, forging the metal into propeller shape while in a heated condition, and which shape is formed with a hub portion, and then gradually deforming the metal of the hub to provide a recess extending axially of the blade and an outwardly extending flange.

28. The method of making a propeller blade which consists in heating a metal casting to a workable condition, rolling out the metal while heated, forging the metal into propeller shape while in a heated condition, and which shape is formed with a hub portion, confining the hub portion in a die, and then piercing the hub axially of the blade with a piercing tool to upset the metal to fill the die.

29. The method of making a propeller blade which consists in heating a metal casting to a workable condition, rolling out the metal while heated, forging the metal into propeller shape while in a heated condition, and which shape is formed with a hub portion, confining the hub portion in a die, and then piercing the hub with a piercing tool to upset the metal into the die, and repeating said confining and piercing operations with differently sized dies and piercing tools to gradually change the shape of the hub portion into its final form.

30. In propeller manufacture, the method of heating a billet of an aluminum base alloy, rolling out the block while heated by a series of rolling operations, which gradually develop the blade in its rough shape, reheating the blade, forging the reheated blade to provide a substantially finished blade portion and a hub portion, and then deforming the hub portion by piercing operations which upset the metal into a hub form having a flattened recess extending axially of the blade.

31. The method of making a propeller from an aluminum base alloy which consists in working

an ingot of the alloy into billet form, rolling out the billet while heated into the general shape of a propeller, further shaping the propeller by forging while heated, working the hub portion into its ultimate form by piercing operations, finishing by operations including cleaning, sizing and trimming, and then heat treating the shaped propeller.

80

32. The method of making a propeller from an aluminum base alloy which consists in rolling an ingot of the alloy into billet form, heating the billet to a workable condition, gradually working the billet while heated into the general shape of a propeller by a series of rolling out operations, further shaping the partially shaped article by forging operations carried out while the metal is rendered workable by heating, finishing by steps comprising sizing, cleaning and trimming, heat treating, and finally finishing by methods including polishing.

85

33. The method of making a propeller from an aluminum base alloy which consists in rolling an ingot of the alloy into billet form, heating the billet to a workable condition, gradually working the billet while heated into the general shape of a propeller by a series of rolling out operations, further shaping the partially shaped article by a series of forging operations, and finishing by steps including sizing and trimming.

90

34. In the manufacture of propellers, the process which consists of forming a substantially cylindrical billet of a cross sectional size providing sufficient metal to carry the forces to which a finished propeller blade is subjected at or near the root portion of the blade, working one end and the major portion of the billet into blade shape and upsetting the opposite end of the billet to form a homogeneous enlargement thereof of greater diameter than the initial diameter of the billet and to work said last mentioned end of the billet to improve the properties thereof.

105

35. In the manufacture of propellers, the process which consists of forming a substantially cylindrical billet of a cross sectional size providing sufficient metal to carry the forces to which a finished propeller blade is subjected at or near the root portion of the blade, working one end and the major portion of the billet into blade shape and radially spreading the opposite end of the billet by an upsetting operation to form an enlargement thereon of greater external diameter than the initial diameter of the billet and to improve the properties of said end of the billet.

110

ALFRED A. HANDLER.

115

120

125

130

135

55

60

140

65

145

70

150

75